

## UNITED STATES PATENT OFFICE

2,073,492

## ORE FLOTATION

Philip A. Ray, Wilmington, Del., assignor to Hercules Powder Company, Wilmington, Del., a corporation of Delaware

No Drawing. Application March 16, 1935, Serial No. 11,439

4 Claims. (Cl. 209—166)

This invention relates to the separation of minerals and the concentration of ores by flotation processes and is particularly directed to the separation and concentration of ores carried out with 5 the utilization of certain organic sulfur compounds as flotation agents or collectors.

According to the present invention the separation of minerals and the concentration of ores by means of the flotation operation is carried out 10 with the aid of a sulfur-containing terpene compound, in particular a terpene mercaptan or thioalcohol. It has been found in accordance with this invention that by the use of these sulfur derivatives of terpene compounds as agents 15 or collectors in the flotation processes better recovery and higher grade concentrations can be obtained.

The flotation agents or collectors employed in the process of flotation in accordance with the 20 present invention may be classified as sulfur-containing terpene compounds or sulfur derivatives of terpene compounds, as, for example, terpene mercaptans or thioalcohols, terpene sulfides or thioethers and terpene di- and polysulfides. 25 These sulfur derivatives of terpene compounds may be prepared, for example, by the treatment of an unsaturated terpene compound with hydrogen sulfide (as is more fully described in an application Serial No. 713,304, filed February 28, 1934, 30 by Joseph N. Borglin and Emil Ott) or by the treatment of halogen derivatives of terpene compounds with alkali sulfides or hydrosulfides (as is disclosed more fully in an application Serial No. 25,427, filed June 7, 1935 by Emil Ott). By 35 variations in procedure, treatment of various terpene compounds in the manner stated above will produce terpene mercaptans, terpene sulfides or thioethers, or terpene-di- and polysulfides. Under usual conditions of procedure all of these 40 various sulfur derivatives will be produced simultaneously in varying amounts, the amount of each being dependent upon the particular conditions of the reaction. Since all these sulfur derivatives of terpene compounds are effective in the process of flotation in accordance with this invention it is not necessary to effect any separation of the mixture produced. However, terpene mercaptans or thioalcohols are the preferred flotation collectors in accordance with this invention, and it will accordingly be desirable that the mixed reaction product contains as large a portion of mercaptans as possible.

In addition to the processes discussed above for the production of sulfur derivatives of terpene compounds, it will be appreciated by the art

that these compounds can be made by other processes. It will therefore be understood that in accordance with the present invention it is contemplated to use sulfur derivatives of sulfides and terpene di- and polysulfides, however produced.

In particular, the present invention contemplates the employment as flotation agents or collectors of sulfur derivatives of pinene, alpha-terpineol, and of a so-called paramenthane cut (a terpene cut boiling within about the range 163° C. to 180° C. and comprising, in addition to small amounts of paramenthane, dipentene, terpinolene and terpinene), since the sulfur derivatives of these terpene compounds, and especially the mercaptans, are exceedingly efficient collectors in flotation processes. The sulfur derivatives of other terpene compounds such as, for example, dipentene, terpinene, terpinolene, etc., can also be used to advantage in the flotation process in accordance with this invention, although they are somewhat inferior in action to the pinene, paramenthane cut and alpha-terpineol products. In carrying out the flotation process the flotation collectors may be incorporated with the ore or mineral pulp in any suitable manner and at any suitable time, for example, they may be introduced in the free state or as salts into the mill in which the ore is being ground, or it may be dissolved, suspended or dispersed in any suitable solvent or dispersing agent, as, for example, the usual flotation oils, such as pine oil, etc., or in water or alkaline reagent, and the resulting suspension, solution or dispersion may be incorporated with the ore or ore pulp. Desirably, the flotation collectors in accordance with this invention will be used in conjunction with frothing agents, as, for example, pine oil, customarily employed in flotation processes.

The process in accordance with this invention can be carried out in any apparatus customarily used for the flotation treatment of ores.

The amount of flotation collector required to be used in the flotation process will vary depending upon the character and composition of the ore, upon the particular flotation collector employed and upon various other variable factors of the flotation process, usually from 0.02 to 5.0 pounds per ton of dry ore will be employed. These quantities are in no way limiting, however, and greater or smaller amounts can be used if desired.

The present invention is further illustrated by the following specific examples of procedure in accordance therewith. In the following examples comparative results are given for processes involving the use of flotation collectors in ac-

cordance with the present invention, such collectors being grouped under the designation "New"; and for processes involving the use of flotation collectors hitherto used in the art, such 5 collectors being grouped under the designation "Old":

**EXAMPLE I**  
**Copper ore**

10 265 g. of copper ore were screened through a 40 mesh screen. The oversize was ground in a ball mill during ten minutes with 250 cc. of water. The ground ore was screened through a 40 mesh screen, and the fines combined. The excess 15 water was decanted from the ore and the latter washed into the flotation machine. To the ore pulp was added 5 cc. of a 1% lime slurry (0.4 #/ton ore), 10 cc. of a 0.1% aqueous solution of sodium cyanide (0.08 #/ton ore), Yarmor F pine 20 oil (0.4 #/ton ore), 3 cc. of a 1% solution (vol.) of the collector under test (0.24 #/ton ore). The time of flotation was ten minutes. The results follow:

| 25         | Collector                     | Percent Cu in concentrate | Percent recovery |
|------------|-------------------------------|---------------------------|------------------|
| <i>New</i> |                               |                           |                  |
| 30         | Pinene mercaptan (9.1% S)     | 24.70                     | 76.6             |
|            | Pinene mercaptan (17.7% S)    | 23.05                     | 75.8             |
|            | Terpineol mercaptan (14.6% S) | 27.65                     | 69.3             |
| <i>Old</i> |                               |                           |                  |
| 35         | Ethyl mercaptan               | 28.83                     | 57.8             |
|            | Benzyl mercaptan              | 23.00                     | 55.0             |
|            | Amyl mercaptan                | 26.2                      | 74.7             |
|            | Potassium ethyl xanthate      | 24.40                     | 72.7             |
|            | Mixed amyl xanthates          | 21.05                     | 85.1             |

**EXAMPLE II**  
**Zinc ore**

40 250 gms. of zinc ore and 250 cc. of water were charged into the ball mill and ground twelve minutes. The contents were discharged onto a 60 mesh screen and washed through. The oversize was rejected. The excess water was decanted and the ore washed into the flotation machine. 45 10 cc. of 1% copper sulfate were added (0.8 #/ton ore), and 0.7 cc. of a 1% solution of the collector (0.056 #/ton ore) was added. The flotation time was fifteen minutes. The results 50 follow:

| 55         | Collector                                                              | Percent Zn in concentrate | Percent recovery |
|------------|------------------------------------------------------------------------|---------------------------|------------------|
| <i>New</i> |                                                                        |                           |                  |
| 60         | Pinene mercaptan (9.1% S)                                              | 12.10                     | 85               |
|            | Pinene mercaptan (17.7% S)                                             | 10.10                     | 87               |
|            | Terpineol mercaptan (14.6% S)                                          | 16.4                      | 92.7             |
| <i>Old</i> |                                                                        |                           |                  |
|            | Amyl mercaptan                                                         | 18.71                     | 83               |
|            | Butyl xanthate                                                         | 29.00                     | 70               |
|            | Sodium "Aerofloat" (a derivative of sodium diethylthiophosphoric acid) | 14.30                     | 83               |

**EXAMPLE III**  
**Zinc ore**

65 In actual field tests on the flotation of zinc ore using the following agents in the flotation:

| 70 |                    | Pounds per ton of ore |
|----|--------------------|-----------------------|
|    | Ore copper sulfate | 0.5                   |
|    | Ore lime           | 0.10                  |
|    | Ore pine oil       | 0.20                  |
| 75 | Ore collector      | 0.04                  |

the following results were obtained for the respective collectors. In each case the ore was conditioned for three minutes with all the flotation agents and flotation was carried out for seven minutes:

|            | Collector                           | Percent Zn in concentrate | Percent recovery |
|------------|-------------------------------------|---------------------------|------------------|
| <i>New</i> |                                     |                           |                  |
| 10         | Pinene mercaptan                    | 46.60                     | 96               |
|            | Pinene mercaptan (caustic extract)  | 40.20                     | 97               |
|            | Mercaptans from the parmenthane cut | 35.60                     | 96               |
| <i>Old</i> |                                     |                           |                  |
| 15         | Sodium "Aerofloat"                  | 29.40                     | 96               |

Duplicate runs under the same conditions gave the following results in which the amount of zinc recovered in the middlings and tailings is separately set out:

|            | Collector                           | Zinc conc. % Zn | Middling % Zn | Tailing % Zn | Recoveries (respective) |
|------------|-------------------------------------|-----------------|---------------|--------------|-------------------------|
| <i>New</i> |                                     |                 |               |              |                         |
| 25         | Pinene mercaptan                    | 40.20           | 0.17          | 0.09         | 96% 2% 2%               |
|            | Mercaptans from the parmenthane cut | 39.60           | 0.16          | 0.08         | 97% 1% 2%               |
| <i>Old</i> |                                     |                 |               |              |                         |
| 30         | Sodium "Aerofloat"                  | 37.30           | 0.22          | 0.16         | 94% 2% 4%               |

The figures for tailings and middlings indicate that better recovery for fine and coarser zinc, respectively, is obtained. Also, a higher grade 35 concentrate is produced.

**EXAMPLE IV**  
**Copper ore**

In field tests in the flotation of copper ore which had been lime and cyanide treated in the plant, the following results were obtained, using the respective flotation agents set out below. In all cases the ore was conditioned with the reagent for five minutes and floated for thirty minutes:

|            | Collector                | Lbs. per ton of bulk Conc. | Concentrate      | Tailing        | Cu recovered |
|------------|--------------------------|----------------------------|------------------|----------------|--------------|
| <i>New</i> |                          |                            |                  |                |              |
| 50         | Pinene mercaptan         | .022                       | Percent 18.66 Cu | Percent .20 Cu | Percent 96.4 |
| <i>Old</i> |                          |                            |                  |                |              |
| 55         | Potassium ethyl xanthate | .04                        | 12.12 Cu         | .21 Cu         | 96.1         |

It will be apparent from consideration of the examples set forth above that the flotation process in accordance with this invention, using a sulfur derivative of a terpene compound as the flotation collectors, is superior, both in the grade of the concentration and in the amount recovered, to flotation processes heretofore used.

It will be understood that the present invention is applicable to the treatment of various kinds of mineral mixtures, both natural and artificial, which may be concentrated by flotation processes.

It will be further understood that the details and examples hereinbefore set forth are for the purpose of illustration only and are not in limitation of the invention as herein broadly described and claimed.

What I claim and desire to protect by Letters Patent is:

1. A method of effecting the concentration of

minerals by flotation which includes subjecting a mineral pulp to a flotation operation in the presence of a terpene mercaptan.

5. 2. A method of effecting the concentration of minerals by flotation which includes subjecting a mineral pulp to a flotation operation in the presence of a pinene mercaptan.

3. A method of effecting the concentration of

minerals by flotation which includes subjecting a mineral pulp to a flotation operation in the presence of a terpineol mercaptan.

4. A method of effecting a concentration of minerals by flotation which includes subjecting a mineral pulp to a flotation operation in the presence of a terpene thioether. 5

PHILIP A. RAY.